

1

3,829,295  
SINTERED IRON BASED ARTICLES INFILTRATED  
WITH COPPER BASED METALS

Edwin Bruce Farmer and Terence Michael Cadle, Coventry, England, assignors to Brico Engineering Limited, Coventry, England

No Drawing. Filed Oct. 13, 1972, Ser. No. 297,363  
Claims priority, application Great Britain, Oct. 23, 1971,

49,345/71  
Int. Cl. B22f 3/26

U.S. Cl. 29—182.1

6 Claims

ABSTRACT OF THE DISCLOSURE

A sintered metal article including a sintered skeleton having the composition 1.5–2.0% Nickel, 0.3–0.7% Molybdenum, 1–2% Copper, 0.1–0.3% Carbon, not more than 2% of Manganese, Silicon, Sulphur, and Phosphorus together (percentages being by weight), the remainder (apart from impurities and trace elements) being Iron, the sintered skeleton being infiltrated with Copper or Copper-based alloy, and the article being case-hardened.

This invention relates to sintered metal articles and to processes for their manufacture.

According to this invention in one aspect, a sintered metal article includes a sintered skeleton having the composition 1.5–2.0% Nickel, 0.3–0.7% Molybdenum, 1–2% Copper, 0.1–0.3% Carbon, not more than 2% of Manganese, Silicon, Sulphur and Phosphorus together (percentages being by weight), the remainder (apart from impurities and trace elements) being Iron, the sintered skeleton being infiltrated with Copper, or Copper-based alloy, and the article being case hardened.

Preferably the skeleton has substantially 1.75% Nickel, 0.5% Molybdenum, 1.5% Copper, 0.25% Combined Carbon.

According to this invention in another aspect, a process for the manufacture of sintered metal articles includes the steps of producing a sintered skeleton having the composition 1.5–2.0% Nickel, 0.3–0.7% Molybdenum, 1–2% Copper, 0.1–0.3% Carbon, not more than 2% of Manganese, Silicon, Sulphur and Phosphorus together, the remainder (apart from impurities and trace elements) being Iron, infiltrating the skeleton with Copper or Copper-based alloy in an amount between 8% and 25% of the skeleton, and then case-hardening the infiltrated article.

Preferably the sintered skeleton is infiltrated with 14% Copper or Copper-based alloy.

A process for the manufacture of articles in accordance with the invention will now be described by way of example.

A pre-alloy or partial pre-alloy in the form of a powder of less than 100 B.S. mesh size and the following composition is selected:

|              | Percent   |
|--------------|-----------|
| Ni           | 1.5–2     |
| Mo           | 0.3–0.7   |
| Cu           | 1.0–2.0   |
| Mn, Si, S, P | (1)       |
| Fe           | Remainder |

<sup>1</sup> Not exceeding 2% in total.

(all the percentages in the specification are by weight).

This pre-alloy or partial pre-alloy powder is mixed with 0.1–0.3% (of the weight of the pre-alloy powder) of Carbon, in the form of graphite, and preferably with a small percentage e.g. 1% of a suitable lubricant such as Zinc Stearate. The constituents are thoroughly mixed in a suitable mixer.

2

The mixture is then pressed at 30–45 tons/sq. in. in a suitable powder metallurgy press, and sintered in a protective atmosphere, for example, a reducing atmosphere of dried cracked Ammonia or a Carbonaceous atmosphere of Endothermic Gas at a temperature in the range 1090° C.–1120° C. for between 20 and 30 minutes. The lubricant disappears in the sintering process.

The sintered article or skeleton is then infiltrated with Copper or Copper-based alloy in an amount equal to between 8 and 25% of the weight of the article, for example, by placing the article in a suitable mould having walls which extend above the article and placing Copper or Copper-based alloy powder on the article, between the walls. The article is then heated in an oven to a temperature significantly above the melting point of Copper or its alloy, so that all the molten Copper or Copper-based alloy infiltrates into the pores of the article; the time of heating is such as to allow the Copper or Copper-based alloy to infiltrate the article uniformly.

Suitable Copper-based alloys are Copper plus 3% Cobalt, or Copper plus 5% Iron and 5% Manganese.

After infiltration the article is then case-hardened either by Carburising, Carbo-Nitriding or any other known or convenient method of Carbon case-hardening.

In one particular example the pre-alloy powder contained 1.75% Nickel, 0.5% Molybdenum, 1.5% Copper, which was mixed with 0.25% Graphite and 1% Zinc Stearate. After sintering in the above manner the skeleton was impregnated with 14% Copper.

The ultimate tensile strength of the article is shown by the following table:

| Condition                               | UTS, tons/sq. in. |
|-----------------------------------------|-------------------|
| As sintered                             | 27                |
| Sintered and case-hardened              | 46                |
| Sintered, infiltrated and case-hardened | 65                |

It will be seen that, surprisingly, the sintered article after infiltration with Copper as described, followed by case-hardening, has a substantially higher ultimate tensile strength than is obtained by case-hardening without infiltration.

This is contrary to what would be expected; for example, an alloy of the composition 10–20% Cu; 0.1–0.3% C; Mn, Si, P together less than 2%; the remainder Fe, shows the following figures:

| Condition                     | UTS, tons/sq. in. |
|-------------------------------|-------------------|
| As sintered                   | 27                |
| Sintered and case-hardened    | 41                |
| Infiltrated and case hardened | 40                |

Other physical properties of articles made in accordance with the invention have been measured as follows:

|                                    |         |         |
|------------------------------------|---------|---------|
| Density                            | gm./cc. | 7.0–8.0 |
| Transverse rupture modulus         | p.s.i.  | 270,000 |
| Impact strength (unnotched Charpy) | ft. lb. | 27      |

We claim:

1. A sintered metal article consisting of a sintered skeleton infiltrated with copper or copper-based alloy, the skeleton having the composition, in percentages by weight:

|                                                     | Percent         |
|-----------------------------------------------------|-----------------|
| Nickel                                              | 1.5–2.0         |
| Molybdenum                                          | 0.3–0.7         |
| Copper                                              | 1–2             |
| Carbon                                              | 0.1–0.3         |
| Manganese, Silicon, Sulphur and phosphorus together | Not exceeding 2 |
| Iron (with impurities and trace elements)           | 93.0–97.1       |

the skeleton being infiltrated with Copper or Copper-based alloy, and the article being case-hardened after infiltration.

2. A sintered metal article, according to Claim 1, in which the skeleton has substantially 1.75% Nickel, 0.5% Molybdenum, 1.5% Copper, 0.25% Carbon.

3. A sintered metal article, according to Claim 1, in which the infiltrated Copper or Copper-based alloy amounts to 8-25% of the skeleton.

4. A sintered metal article, according to Claim 3, infiltrated with 14% Copper or Copper-based alloy.

5. A sintered metal article, according to Claim 1, which is case-hardened by carburising.

6. A sintered metal article, according to Claim 1, which is case-hardened by carbo-nitriding.

#### References Cited

##### UNITED STATES PATENTS

|           |         |               |       |          |
|-----------|---------|---------------|-------|----------|
| 3,414,391 | 12/1968 | Brab          | ----- | 29—182.1 |
| 3,694,173 | 9/1972  | Farmer et al. | ----- | 29—182.1 |

5

##### FOREIGN PATENTS

|           |         |               |       |          |
|-----------|---------|---------------|-------|----------|
| 1,071,863 | 6/1967  | Great Britain | ----- | 29—182.1 |
| 720,050   | 12/1954 | Great Britain | ----- | 29—182.1 |

10 CARL D. QUARFORTH, Primary Examiner

B. HUNT, Assistant Examiner

U.S. Cl. X.R.

15 29—182.5, 182.7